

# UNITED STATES PATENT OFFICE.

CARVER HIDECKER, OF SAN ANSELMO, CALIFORNIA, ASSIGNOR TO IONE FIRE BRICK COMPANY, OF SAN FRANCISCO, CALIFORNIA, A CORPORATION OF CALIFORNIA.

## FIRE-BRICK.

1,115,429.

Specification of Letters Patent. Patented Oct. 27, 1914.

No Drawing.

Application filed June 8, 1913. Serial No. 771,537.

To all whom it may concern:

Be it known that I, CARVER HIDECKER, a citizen of the United States, residing at San Anselmo, in the county of Marin and State of California, have invented new and useful Improvements in Fire-Brick, of which the following is a specification.

The object of the present invention is to provide a fire brick of great efficiency and comparatively small cost.

Cast and wrought stoves and boiler fire boxes for use with coal are lined with clay linings made in molds and burnt sufficiently to hold their form. These linings are adapted to withstand a heat not exceeding a "smoking" temperature, that is, at which the heat is not sufficient to prevent the formation of smoke. They are composed of flint clays or silica sands together with plastic or potter clays. The flint clays and silica sands fuse only at high temperatures, and the plastic clays, which are used merely to bind said clays, or sands in the forms or bricks, fuse at somewhat lower temperatures. These materials are properly mixed, and a brick formed of the mixture is raised to a temperature between the fusing points of plastic clay and flint clay or silica sands. When allowed to cool, it contracts, and becomes a dense granular mass, and being less porous it possesses a greater resistance than before to the passage of heat. Such a brick when exposed to very great heat is destroyed in the following manner. Heat applied to the exterior of the brick travels along its pores, causing an expansion of the mass, so that the granules in the brick are more accessible to the heat and can to a less degree withstand its action, which therefore proceeds with increased effect, until finally complete disintegration takes place.

As municipal smoke ordinances for the prevention of smoke emission have been put into effect, it has been learned that the prevention of smoke can, in practice, only be secured by preventing its original formation. This can only be done by using very high temperatures in the furnace. As these temperatures are at least 1,000° F. higher than the "smoking" temperature heretofore used, there is a demand for a brick that will resist heat of such high temperatures. Only in a measure has the demand been met. This has been done principally, so far as I am aware, by applying to the surface of the bricks after they are set in furnaces certain

cements, fusible only at a high temperature. The office of these cements is to close the porosity of the granular-mass brick on its surface by a material which will fuse only at a high heat, said cement thus furnishing a very great obstruction to the transmission of the heat into the brick, both by closing the pores in the brick through which the heat might the more easily penetrate and also by providing a surface material which cannot readily be removed by fusion. However there are two principal objections to a brick of this character; first, if the surface becomes fractured its efficiency is lost; second, the cost of applying these cements doubles the cost of the granular-mass brick.

I propose to produce a fire brick which has the combined advantages of the granular-mass brick and the high-temperature cement and at an increase in the cost of only 30 per cent. of the increase by said use of cement. In this brick I propose to use 75 per cent. of non-contracting refractory material, as flint clay, or silica sands, fusing only at a temperature of 2800° F., 10 per cent. of plastic clay, contracting from its original condition after being fused, and fusing at a temperature of 2,500° F., 10 per cent. of shale fusing at 2250° F. and 5 per cent. of practically infusible material, by which is meant one which does not fuse at a temperature below 4,000° F.

A brick of the above materials is made by burning in a kiln at a heat of not less than 2800° F. When cooled from such a temperature it will shrink or be compacted, but it can never again be fused by a furnace heat of less than 3500° F. This result is due to the employment of a practically infusible material combined with a pore-filling material, which practically infusible material offers so great resistance to the passage of heat through the more easily fusible material that the brick cannot become fused at a less temperature than above stated.

Furnace bricks are destroyed by absorption of heat through the pores more readily than through the external surface of the brick. The reason for this is that the external surface of the brick is very small compared with its internal surface around the pores. Hence, if the pores of the brick be filled by a substance which cannot be readily fused, it follows that the brick can only absorb heat through the external surface. The practically in-

fusible material used in the brick is a product of the electric furnace, one such substance being carborundum. I do not confine myself to any special substance, but claim 5 the invention using any practically infusible material.

It will readily be understood from the foregoing description that it is important to proportion the relative sizes of the several 10 materials. The flint clay or silica sands are used in comparatively large particles, while the pore-filling material and the practically non-fusible material are in very fine particles, the object of the latter two being to 15 fill up the voids made by the large particles of refractory material. Furthermore the percentage of the ingredients above described will vary in amounts according to their purity or condition as found in nature.

I claim:—

A fire brick comprising substantially 20 seventy-five per cent. of silicious material fusing only at a temperature of twenty-eight hundred degrees F., ten per cent. of argillaceous material fusing at a temperature 25 of twenty-five hundred degrees F., ten per cent. of shale fusing at twenty-two hundred fifty degrees F., and five per cent. of material which cannot be fused at a temperature below four thousand degrees F. 30

In testimony whereof I have hereunto set my hand in the presence of two subscribing witnesses.

CARVER HIDECKER.

Witnesses:

FRANCIS M. WRIGHT,  
D. B. RICHARDS.